

# United States Patent [19]

Alcorn et al.

[11] 3,779,930

[45] Dec. 18, 1973

[54] FLUIDS

[75] Inventors: **Percival George Ernest Alcorn, Hawthorn; Keith Gordon Neill, Kew, Victoria, both of Australia**

[73] Assignee: **Imperial Chemical Industries of Australia and New Zealand Limited, Melbourne, Victoria, Australia**

[22] Filed: **May 26, 1971**

[21] Appl. No.: **147,231**

[30] Foreign Application Priority Data

Oct. 9, 1970 Australia..... 1507/70  
Oct. 9, 1970 Australia..... 2813/70

[52] U.S. Cl..... 252/77, 252/79

[51] Int. Cl..... C09k 3/00, C10m

[58] Field of Search ..... 252/73, 77, 76, 75, 252/79, 51.5 R, 56 S; 260/484 R, 465.6

[56] References Cited

UNITED STATES PATENTS

|           |        |                |           |
|-----------|--------|----------------|-----------|
| 2,942,033 | 6/1960 | Leis et al.    | 252/404 X |
| 2,200,495 | 5/1940 | Fife           | 252/77 X  |
| 2,520,612 | 8/1950 | Roberts et al. | 252/73 X  |
| 2,886,600 | 5/1959 | Horsley et al. | 252/73 X  |
| 2,998,389 | 8/1961 | White          | 252/73    |
| 3,137,737 | 6/1964 | Emrick et al.  | 252/73 X  |

|           |         |              |                    |
|-----------|---------|--------------|--------------------|
| 3,538,003 | 11/1970 | Lothar       | ..... 252/77       |
| 3,623,987 | 11/1971 | Ker et al.   | ..... 252/79       |
| 2,836,613 | 5/1958  | Heininger    | ..... 252/51.5 R X |
| 2,226,599 | 12/1940 | Zellhoefer   | ..... 260/484 R    |
| 2,350,964 | 6/1944  | Loder et al. | ..... 260/484 R    |
| 3,278,585 | 10/1966 | Baker et al. | ..... 252/79 X     |

FOREIGN PATENTS OR APPLICATIONS

1,188,825 4/1970 Great Britain

Primary Examiner—Leon D. Rosdol

Assistant Examiner—Harris A. Pitlick

Attorney—Cushman, Darby & Cushman

[57] ABSTRACT

New compositions of use as hydraulic fluids comprising a compound of general formula I:



wherein Alk is an alkylene or aralkylene group containing from 1 to 9 inclusive carbon atoms in a straight or branched chain, R<sub>1</sub> and R<sub>2</sub>, separately, is an alkyl, substituted alkyl or aralkyl group containing from 1 to 10 inclusive carbon atoms in a straight or branched chain and n is an integer from 1 to 10 inclusive, said compound having a viscosity at -40° C. of less than 1800 centistokes; and at least one additive.

4 Claims, No Drawings

1  
FLUIDS

This invention relates to hydraulic fluid.

Hydraulic fluids are used in many pressure transmission systems, for example, in hydraulic machinery such as hydraulic presses and rams, and the clutching and braking systems of vehicles. The pressure transmission systems must operate over a wide range of conditions and the hydraulic fluid, to be effective, must not attack the machinery and must also remain a free flowing liquid under the extremes of the external conditions encountered.

The hydraulic brake systems of vehicles such as, for example, motor cars and aeroplanes comprise both metal and rubber parts exposed to the liquid employed as the hydraulic fluid. It is necessary that the hydraulic fluid does not attack either the metal or the rubber parts of the brake system, either at ordinary temperatures or at the elevated temperatures such as those caused by prolonged application of the brakes. The hydraulic fluid must also be unaffected by the low temperatures found during cold weather or in the case of aeroplanes in high altitude flight. This means that the freezing point should be below those temperatures likely to be encountered under operating conditions, and in addition the viscosity of the fluid should not increase under these conditions to such an extent that the easy working of the brakes is hindered. It is also essential that the hydraulic fluid should have a high boiling point so as to ensure that the hydraulic fluid will not vaporize and cause vapour locks under operating conditions. The hydraulic fluid should also have a low rate of vaporization and also sufficient lubricating properties to lubricate the moving parts of the system.

Conventional hydraulic fluids normally comprise a major proportion of polyalkylene glycols, and/or polyalkylene glycol monoethers together with minor proportions of various additives.

In practice, it is found that hydraulic brake fluids based on polyalkylene glycols and/or polyalkylene glycol monoethers are hygroscopic and in the passage of time water is absorbed from the atmosphere and the boiling point steadily falls. It is not uncommon, for example, for a brake fluid, after several months service, to be found to contain about 1 percent of water and, on prolonged service, up to 3 percent of water may be found in such fluids.

It is important for a hydraulic brake fluid to retain a high boiling point throughout its useful life, since a reduction in boiling point may result in the formation of vapour locks with consequent failure of the braking system. So as to avoid this possibility, it is usual for current brake fluids based on polyalkylene glycols and/or polyalkylene glycol monoethers, to be changed at least once every two years, so that moisture is not allowed to accumulate in the hydraulic fluid. It is desirable that the boiling point of a fluid should not be allowed to fall below about 300°F.

There is a need for hydraulic fluids of improved properties. In the past, hydraulic fluids for typical "heavy duty" braking systems had a boiling point of about 400°F, but with generally increased severity of operation, especially in vehicles fitted with disc brakes, there is now a need for hydraulic fluids having even higher boiling points; and fluids boiling at a temperature greater than 500°F. are desired.

## 2

We have now found that hydraulic fluids comprising certain diethers have the desirable properties of high boiling point, low freezing point, acceptable rubber swell, and low hygroscopicity.

5 Accordingly we provide a hydraulic fluid comprising at least one diether of general formula I:



10

wherein Alk is an alkylene or aralkylene group containing from 1 to 9 inclusive carbon atoms in a straight or branched chain,  $R_1$  and  $R_2$ , separately, is an alkyl, substituted alkyl or aralkyl group containing from 1 to 10 inclusive carbon atoms in a straight or branched chain and  $n$  is an integer from 1 to 10 inclusive, said diether having a viscosity of less than 1800 centistokes at -40°C.; and at least one additive.

15 Satisfactory hydraulic fluids may be obtained, for example, when  $R_1$  is alkyl, aralkyl, beta-cyanoalkyl or beta-alkoxycarbonylalkyl and  $R_2$  is beta-cyanoalkyl or beta-alkoxycarbonylalkyl.

20 Suitable diethers used in our invention may be prepared by known means from condensates of ethylene oxide, propylene oxide, butylene oxide, styrene oxide, alpha-methyl styrene oxide or mixtures thereof, with water or an alkyl or aralkyl alcohol containing from 1 to 10 inclusive carbon atoms. Among suitable condensates, there may be mentioned, for example, ethylene

25 glycol, ethylene glycol monomethylether, ethylene glycol monoethyl ether, diethylene glycol, diethylene glycol monomethyl ether, diethylene glycol monobutyl ether, triethylene glycol, triethylene glycol monomethyl ether, triethylene glycol monoethyl ether, propylene glycol, propylene glycol monomethyl ether, propylene glycol monoethyl ether, dipropylene glycol, dipropylene glycol monobutyl ether, dipropylene glycol monoethyl ether, tripropylene glycol, tripropylene glycol monomethyl ether and tripropylene glycol monoethyl ether.

30 35 40 45 We have found under certain circumstances that the use of a mixture of diethers in our hydraulic fluids is beneficial. Thus the inclusion of a proportion of diethers of formula I, wherein  $n$  is an integer from 20 to 100 inclusive, in our hydraulic fluids improves the lubricating characteristics of our hydraulic fluids.

Particularly suitable hydraulic fluids may be prepared when  $R_2$  is a beta-cyanoalkyl group. Such a group may be introduced into the diethers used in our hydraulic fluid by reacting suitable condensates as illustrated above with beta-cyano-olefines such as for example acrylonitrile or methacrylonitrile.

50 55 Accordingly we provide a hydraulic fluid comprising a diether of general formula II:



II

60 65 wherein Alk is an alkylene or aralkylene group containing from 1 to 9 inclusive carbon atoms in a straight or branched chain,  $R$  is an alkyl, substituted alkyl or aralkyl group containing from 1 to 10 inclusive carbon atoms in a straight or branched chain,  $R_3$  and  $R_4$ , separately, is a hydrogen atom or an alkyl group containing from 1 to 4 inclusive carbon atoms and  $n$  is an integer from 1 to 10 inclusive, said diether having a viscosity

of less than 1800 centistokes at  $-40^{\circ}\text{C}$ ; and at least one additive.

The additives are selected from those known in the art to be effective for improving the properties of hydraulic fluids. Hydraulic fluids normally contain amongst other ingredients various additives such as lubricating additives, corrosion inhibitors, antioxidants and the like. The exact nature of the additives required to obtain a hydraulic fluid of optimum performance may be found by the methods normally used by those skilled in the art.

Lubricity additives which may be used in our invention include, for example, 'Ucon' lubricants (Trade Mark for polyalkylene glycols), alkoxylated castor oil or borate esters. Certain of the diethers described hereinabove may also be used as lubricity additives. Corrosion inhibitors which may be used in our invention include, for example, heterocyclic nitrogen containing compounds, amines or derivatives of amines, organic phosphates or certain inorganic salts known in the art. Certain compounds may be used both as corrosion inhibitors and as lubricity additives, these include, for example, orthophosphate salts of primary or secondary aromatic amines, dialkyl citrates, aliphatic dicarboxylic acids and esters thereof. Antioxidants which may be used in our invention include, for example, diaryl amines, compounds of the class commonly known as hindered phenols and heterocyclic compounds known in the art.

The invention is illustrated but by no means limited by the following examples in which all parts are parts by weight unless otherwise stated.

#### EXAMPLE 1

Hydraulic fluid A according to this invention was prepared by mixing 99.7 parts of 1-(2-methoxyethoxy)-2-(2-cyanoethoxy)-ethane having a viscosity at  $-40^{\circ}\text{C}$  of 400 centistokes with 0.3 parts of 'Topanol' A (Trade Mark of Imperial Chemical Industries Limited for 2-tert-butyl-6-methyl-p-cresol).

Comparative hydraulic fluid B not of our invention, was prepared by mixing diethylene glycol monomethyl ether (99.7 parts) with 'Topanol' A (0.3 parts).

Hydraulic fluid C was prepared by mixing 99.7 parts of 1-(2-methoxyethoxy)-2-(2-cyanopropoxy)-ethane

having a viscosity at  $-40^{\circ}\text{C}$  of 260 centistokes with 0.3 parts of 'Topanol' A.

Hydraulic fluid D was prepared by mixing 99.7 parts of tripropylene glycolmethyl ether beta-methyl-beta-cyanoethyl ether having a viscosity at  $-40^{\circ}\text{C}$  of 1570 centistokes with 0.3 parts of 'Topanol' A.

The total reflux boiling point, freezing point (non-stirrable) rubber swell and the water uptake of hydraulic fluids A, B, C and D were measured. The water uptake was measured in the following manner. A weighed sample (5 g) of the hydraulic fluid was exposed, in a shallow dish, in a humidity chamber under a constant atmosphere of 75 percent relative humidity at  $75^{\circ}\text{F}$ . The samples were weighed after being kept under these conditions for 96 hours. The water uptake was the percentage increase in weight per unit weight of the original sample.

The rubber swell was measured by measuring the increase of diameter in inches of the base of a styrene rubber piston cup after the cup had been immersed in a hydraulic fluid at a temperature of  $120^{\circ}\text{C}$  for 70 hours.

The rubber cups used in this test were of a standard size having a base diameter in the range 2.77 cm to 2.8 cm. inclusive. The results obtained are tabulated in Table 1.

TABLE 1

| Hydrau-<br>lic<br>Fluid | Total<br>reflux<br>boiling<br>point °F | Freezing<br>point<br>(non-<br>stirrable)<br>°C | Water<br>uptake | Rubber<br>swell |
|-------------------------|----------------------------------------|------------------------------------------------|-----------------|-----------------|
| A                       | 543                                    | <-76                                           | 4.6             | + 0.013         |
| B                       | 381                                    | <-94                                           | 18.1            | + 0.005         |
| C                       | 528                                    | <-65                                           | 2.9             | + 0.045         |
| D                       | 575                                    | -61                                            | 2.3             | + 0.103         |

#### EXAMPLE 2

A series of hydraulic fluids were prepared by mixing separately 99.7 parts of the compounds whose structure is shown in Table 2 with 0.3 parts of 'Topanol' A.

The boiling point, water uptake, freezing point, and rubber swell of the compositions were measured and the results are shown in Table 2. The water uptake and the rubber swell were measured by the method of Example 1.

TABLE 2

| Structure of compound                                                                                                                                                                                           | Viscosity of compound in centistokes at $-40^{\circ}\text{C}$ . | Total reflux boiling point of hydraulic fluid (°F.) | Freezing point (non-stirrable) of hydraulic fluid (°C.) | Water uptake of hydraulic fluid | Rubber swell of hydraulic fluid |
|-----------------------------------------------------------------------------------------------------------------------------------------------------------------------------------------------------------------|-----------------------------------------------------------------|-----------------------------------------------------|---------------------------------------------------------|---------------------------------|---------------------------------|
| $\text{CH}_3-\text{O}(\text{CH}_2)_2\text{O}-\text{CH}_2-\text{CH}_2-\text{CN}$                                                                                                                                 | 61.2                                                            | 439                                                 | <-60                                                    | 5.0                             | + 0.027                         |
| $\text{CH}_3\text{CH}_2-\text{O}-\text{CH}_2-\text{CH}_2-\text{O}-\text{CH}_2-\text{CH}_2-\text{CN}$                                                                                                            | 88.6                                                            | 453                                                 | <-60                                                    | 4.6                             | + 0.013                         |
| $\text{CH}_3\text{CH}_2-\text{O}-(\text{CH}_2-\text{CH}_2-\text{O})_2-\text{CH}_2-\text{CH}_2-\text{CN}$                                                                                                        | 540                                                             | 534                                                 | <-60                                                    | 3.9                             | + 0.027                         |
| $\text{CH}_3-(\text{CH}_2)_3-\text{O}-(\text{CH}_2-\text{CH}_2-\text{O})_2-\text{CH}_2-\text{CH}_2$<br>CN                                                                                                       | 530                                                             | 584                                                 | <-60                                                    | 2.3                             | + 0.079                         |
| $\text{CH}_3-\text{O}-\text{CH}_2-\text{CH}(\text{CH}_3)-\text{O}-\text{CH}_2-\text{CH}_2-\text{CN}$                                                                                                            | 207                                                             | 533                                                 | <-72                                                    | 3.9                             | + 0.032                         |
| $\text{CH}_3-\text{O}-(\text{CH}_2\text{CH}_2\text{O})_{2.7}-\text{CH}_2-\text{CH}_2-\text{CN}$<br>$\text{CH}_3-\text{CH}_2\text{O}-(\text{CH}_2-\text{CH}_2-\text{O})_{2.7}-\text{CH}_2-\text{CH}_2-\text{CN}$ | 910<br>1190                                                     | 550<br>560                                          | -60<br>-57                                              | 8.6<br>7.6                      | + .013<br>+ .040                |
| $\text{CH}_3-\text{O}-\text{CH}_2-\text{CH}_2-\text{O}-\text{CH}_2-\text{CH}_2$<br>C=O<br>$\text{CH}_3-\text{O}-\text{CH}_2-\text{CH}_2-\text{O}$                                                               | 208                                                             | 518                                                 | <-65                                                    | 3.0                             | + 0.087                         |

TABLE 2—Continued

| Structure of compound                                                                                                                                              | Viscosity of compound in centistokes at -40°C. | Total reflux boiling point of hydraulic fluid (°F.) | Freezing point (non-stirrable) of hydraulic fluid (°C.) | Water uptake of hydraulic fluid | Rubber swell of hydraulic fluid |
|--------------------------------------------------------------------------------------------------------------------------------------------------------------------|------------------------------------------------|-----------------------------------------------------|---------------------------------------------------------|---------------------------------|---------------------------------|
| $\text{CH}_3-\text{O}-\text{CH}_2-\text{CH}_2-\text{O}-\text{CH}_2-\text{CH}_2$   | 120                                            | 456                                                 | < -65                                                   | 3.2                             | + .160                          |
| $\text{CH}_3-\text{O}-\text{CH}_2-\text{CH}-\text{O}$                             |                                                |                                                     |                                                         |                                 |                                 |
| $\text{CH}_3-\text{O}-\text{CH}_2-\text{CH}_2-\text{O}-\text{CH}_2-\text{CH}_2$   | 257                                            | 545                                                 | < -65                                                   | 6.6                             | + .073                          |
| $\text{CH}_3-\text{O}-\text{(CH}_2-\text{CH}_2-\text{O})_2$                       |                                                |                                                     |                                                         |                                 |                                 |
| $\text{CH}_3\text{O}(\text{CH}_2-\text{CH}_2\text{O})_2-\text{CH}_2-\text{CH}_2$  | 620                                            | 595                                                 | < -65                                                   | 5.7                             | + .072                          |
| $\text{CH}_3-\text{O}-\text{(CH}_2-\text{CH}_2-\text{O})_2$                       |                                                |                                                     |                                                         |                                 |                                 |

### EXAMPLE 3

A hydraulic fluid was prepared by mixing diethylene-glycol methylether 2-cyanoethyl ether (80 parts) with "Ucon" 50 HB660 (20 parts) ("Ucon" 50 HB660 is a Trade Mark for polyalkylene glycols).

The hydraulic fluid was found to have a viscosity at  $-40^{\circ}\text{C}$  of 1640 centistokes and the rubber swell as measured in Example 1 was 0.018.

#### EXAMPLE 4

A hydraulic fluid was prepared by mixing diethylene-glycol ethylether 2-cyanoethyl ether (60 parts), diethylene-glycol n-butyl ether 2-cyanoethyl ether (20 parts) and "Ucon" 50 HB260 (20 parts). ("Ucon" 50 HB260 is a Trade Mark for polyalkylene glycols).

The hydraulic fluid was found to have a viscosity at  $-40^{\circ}\text{C}$  of 1350 centistokes and the rubber swell measured by the method of Example 1 was 0.041.

**EXAMPLE 5**

A hydraulic fluid was prepared by mixing diethylene-glycol methylether 2-cyanoethyl ether (60 parts), diethylene-glycol n-butylether 2-cyanoethyl ether (20 parts) and "Ucon" 50 HB260 (20 parts).

The hydraulic fluid was found to have a viscosity at  $-40^{\circ}\text{C}$  of 1090 centistokes and the rubber swell measured by the method of Example 1 was 0.029.

**EXAMPLE 6**

A hydraulic fluid was prepared by mixing diethylene-glycol methylether 2-cyanoethyl-ether (50 parts) with propylene-glycol bis-2-cyanoethyl-ether (50 parts).

The hydraulic fluid was found to have a viscosity at  $-40^{\circ}\text{C}$  of 1290 centistokes and the rubber swell measured by the method of Example 1 was 0.007.

**EXAMPLE 7**

A hydraulic fluid was prepared by mixing diethylene-glycol ethylether 2-cyanoethylether (60 parts) with propyleneglycol bis-2-cyanoethyl ether (40 parts).

The hydraulic fluid was found to have a viscosity at  $-40^{\circ}\text{C}$  of 1500 centistokes and the rubber swell measured by the method of Example 1 was 0.012.

### EXAMPLE 8

A hydraulic fluid was prepared by mixing diethylene-glycol methylether 2-cyanoethyl-ether (79.7 parts) "Ucon" 50 HB660 (20 parts), 'Topanol' A (0.3 parts) benzotriazole (0.02 parts), di-n-butylamine (0.30 parts) and m-dinitro-benzene (0.05 parts).

The hydraulic fluid was found to have the properties shown in Table 3.

TABLE 3

|                                           |                  |
|-------------------------------------------|------------------|
| Total reflux boiling point                | 522°F            |
| viscosity                                 | 1640 centistokes |
| pH                                        | 10.9             |
| rubber swell                              | + 0.018          |
| loss in weight by evaporation<br>at 100°C | 72%              |

The degree of rubber swell was measured by the method of Example 1.

The hydraulic fluid was found to have acceptably low corrosive action on tinned iron, steel, cast iron, brass, copper and aluminium.

We claim:

1. In a method for transmitting pressure using a hydraulic fluid, the improvement wherein said hydraulic fluid consists essentially of one or more diethers of general formula:



wherein Alk is an alkylene group containing from 1 to 4 inclusive carbon atoms in a straight or branched chain,  $R_1$  is alkyl containing from 1 to 10 inclusive carbon atoms in a straight or branched chain,  $R_2$  is a beta-cyanoalkyl group containing from 1 to 10 inclusive carbon atoms and  $n$  is from 1 to 10 inclusive, said diether having a viscosity of less than 1800 centistokes at  $-40^\circ C$ .

2. A method according to claim 1 wherein the beta-cyanoalkyl  $R_2$  is the group  $-\text{CHR}_3-\text{CHR}_4-\text{CN}$  wherein  $R_3$  and  $R_4$  are each selected from the group consisting of hydrogen and alkyl containing from 1 to 4 inclusive carbon atoms.

3. A method according to claim 2 wherein each of  $R_3$  and  $R_4$ , separately, is hydrogen or methyl.

4. A method according to claim 1 wherein the diether

(oxy)-2-(2-cyano-

UNITED STATES PATENT OFFICE  
CERTIFICATE OF CORRECTION

Patent No. 3,779,930 Dated December 18, 1973

Inventor(s) Percival George Ernest Alcorn et al

It is certified that error appears in the above-identified patent and that said Letters Patent are hereby corrected as shown below:

In the heading, the Foreign Application Priority data for Australian Application No. 1507/70 should read --June 16, 1970--.

Signed and sealed this 9th day of July 1974.

(SEAL)  
Attest:

McCOY M. GIBSON, JR.  
Attesting Officer

C. MARSHALL DANN  
Commissioner of Patents